

# UNITED STATES PATENT OFFICE.

THOMAS MORRISON, OF BRADDOCK, PENNSYLVANIA.

## METHOD OF ROLLING FLANGED SECTIONS.

SPECIFICATION forming part of Letters Patent No. 722,605, dated March 10, 1903.

Application filed April 23, 1902. Serial No. 104,407. (No specimens.)

*To all whom it may concern:*

Be it known that I, THOMAS MORRISON, of Braddock, in the county of Allegheny and State of Pennsylvania, have invented a new and useful Method of Rolling Flanged Sections, of which the following is a full, clear, and exact description.

My invention relates to the rolling of flanged sections, and more especially to the process set forth in my Patent No. 654,071, dated July 15, 1900.

In improving the quality of flanged shapes, especially railway-rails, according to the method of my said patent the shapes have been cooled down before finishing them in the final pass of the mill, and the present invention is designed to make it easier for the operator to bring the different sections to substantially the same temperature before final rolling, and thus to obtain more uniform results. The use of pyrometers in this connection has been found to be difficult.

My invention is based upon the discovery that the heat of each section before rolling in the final pass or passes can be ascertained relatively to that of other sections by comparing the amount of shrinkage after the rails or other sections have been cut from the long rolled section, and by setting the hot saws at a fixed distance apart the straighteners by reporting any slight change in the final length of the rail can direct the operator controlling the group of cooling rails or other sections, so that he is enabled to obtain substantially uniform results.

To illustrate the principle of my invention, I will describe the following as an example: I have discovered that I can obtain more accurate results by cooling the sections to such

a temperature before final rolling that in an 40 eighty-five-pound rail the rail shall be cut not over five and three-fourths ( $5\frac{3}{4}$ ) inches longer than thirty (30) feet to give the desired thirty-foot rail. In such case, therefore, the hot saws used to sever the long rolled 45 section into rail lengths are set at a fixed distance apart, which is less than five and three-fourths ( $5\frac{3}{4}$ ) inches and is preferably five and five-eighths ( $5\frac{5}{8}$ ) inches longer than the thirty-foot length of the rail, and any slight 50 variation in the final length of the rails after cooling can be reported by the straighteners to the operator controlling the group of rails being cooled before the final pass, and he will hold them a slightly greater or less length 55 of time upon the cooling-bed, whichever is necessary in order to correct such slight variation.

It will be understood that the length of the section will be varied according to the weight 60 per pound and the final length desired, &c.

I claim—

The method herein described of treating flanged metal sections during the rolling thereof, consisting in cooling the flanged sections before the final pass, finish-rolling the section in the final pass or passes, cutting said finished section into fixed lengths and controlling the time interval of said cooling by measuring the rail with relation to the 70 length to which it will contract when cold; substantially as described.

In testimony whereof I have hereunto set my hand.

THOMAS MORRISON.

Witnesses:

G. E. F. GRAY,  
J. E. MITCHELL.